

## UNITED STATES PATENT OFFICE.

HERMANN WAGNER, OF SODEN-ON-THE-TAUNUS, AND HEINZ EICHWEDE AND ERICH FISCHER, OF HOCHST-ON-THE-MAIN, GERMANY, ASSIGNEES TO GRASSELLI DYE-STUFF CORPORATION, OF NEW YORK, N. Y., A CORPORATION OF DELAWARE.

## PROCESS OF DYEING MIXED TEXTILE GOODS.

No Drawing. Application filed January 28, 1926, Serial No. 84,501, and in Germany February 7, 1925.

It is already known that a number of pyrazolone azo dyestuffs possess a certain affinity for the silk fibre. However this affinity is not sufficient to dye the silk fibre 5 when mixed with wool fibre, just as intensely as the wool fibre.

Now we have found that a certain group of pyrazolone azo dyestuffs are distinguished from the said known dyestuffs by an increased affinity for the silk fibre, which 10 affinity, when suitable combinations of dyestuffs are selected, may be enhanced so much that the silk fibre as well as the wool fibre are evenly dyed in a single bath. The dyestuffs in question are such as contain in the diazo component or in the coupling component, or in both components simultaneously, one or more carboxylic acid ester groups. The dyeings obtainable thereby, 15 which vary from yellow to orange, are distinguished by very good properties as to fastness. The wool and silk fibres are dyed even tints. Regarding the degree of the affinity of the dyestuffs for the silk fibre as 20 compared with that for the wool fibre it should be considered that it is advantageous that the combinations of dyestuffs to be selected do not contain more acid groups—such as sulfo- or free carboxylic groups— 25 than are necessary for rendering the dyestuff soluble in the usual dye bath.

The following examples illustrate our invention:

(1) 1 kg. of material mixed of wool- and 35 silk fibres is dyed in an appropriate manner in a dyebath containing 20 gr. of the dyestuff: ortho - chloraniline  $\longrightarrow$  1-(4'-sulfo-

phenyl-5-pyrazolone-3-carboxylic ethyl ester, while adding 10% of sodium sulfate and 4% 40 of sulfuric acid. The dyeing thus obtained is not only distinguished for its great fastness but also for the fact that the wool- as well as the silk fibres are dyed evenly and in an equal shade.

(2) By substituting for the dyestuff indicated in Example 1 an equal quantity of the dyestuff: ortho-aminobenzoic acid ethyl ester  $\longrightarrow$  1-(4'-sulfo-phenyl)-3-methyl-5-pyrazolone, there is also obtained a very pure yellow dyeing, the silk fibre as well as the wool fibre being dyed a tint of even shade and intensity.

(3) When using the dyestuff: m-amino-benzoic acid ethyl ester  $\longrightarrow$  1-(4'-sulfo-

phenyl)-5-pyrazolone-3-carboxylic acid ethyl ester and operating the dyeing as indicated in Example 1 there are also obtained on the said material very even tints.

The dyestuff combinations specified in the foregoing examples are only to be regarded as representatives of the respective groups. They may, of course, be largely varied both in the diazo component and in the coupling component.

Thus, for instance the pyrazolone compound mentioned in Examples 1 and 3, may be replaced by the following combinations:

(1) 1-(2'-sulfo-phenyl)-5-pyrazolone-3-carboxylic acid ester.

(2) 1-(2'5'-dichloro-4'-sulfo-phenyl)-5-pyrazolone-3-carboxylic acid ester.

(3) 1-(2'-chlor-5'-sulfo-phenyl)-5-pyrazolone-3-carboxylic acid ester.

(4) 1-(2'-methyl-6'-chloro-4'-sulfo-phenyl)-5-pyrazolone-3-carboxylic acid ester.

(5) 1-(2'-methyl-4'-methyl-5'-sulfo-phenyl)-5-pyrazolone-3-carboxylic acid ester.

Furthermore in the diazo component named in Example 1 the ortho-chloroaniline may for instance be replaced by: aniline, 80 ortho-meta- and para-toluidine or the like. However it is preferable that the diazo compounds do not contain any sulfo group, because in this case the wool fibre is dyed more deeply than the silk fibre. In any case, however, the dyestuffs of this kind are distinguished from the analogous dyestuffs in which the sulfo-phenyl-pyrazolone-carboxylic acid is not esterified, by the property of dyeing the silk fibre in mixed material more 85 deeply.

For the pyrazolone-sulfonic acid mentioned in Example 2 may be substituted any other sulfo-aryl-3-methyl-5-pyrazolone but no sulfo-phenyl-5-pyrazolone-3-carboxylic acid.

In like manner, the diazo compounds mentioned in Examples 2 and 3 may be replaced by any other amino-aryl-carboxylic acid ester, for instance by 4-nitro-2-aminobenzoic acid methyl ester etc.

It is to be understood that, in the foregoing description, the arrow ( $\longrightarrow$ ) is used to indicate the linkage of two components of an azo-dyestuff. Thus in the case of the dyestuff o-chlor-aniline  $\longrightarrow$  1-(4'-sulfo-phenyl)-5-pyrazolone-3-carboxylic ethyl ester the arrow indicates that 6-chlor-aniline has been diazotized and the diazo compound

so formed has been coupled with the particular pyrazolone compound stated. This use of the arrow is described by Georgievics & Grandmougin, "A Text-Book of Dye Chemistry", translated from the fourth German edition by F. A. Mason, 1920, pages 87 and 88.

We claim:

1. Process which comprises dyeing mixed textile goods made of wool and silk fibers with a pyrazolone-azo dyestuff containing at least one carboxylic acid ester group in the dyestuff molecule, said pyrazolone-azo dyestuff containing no free carboxylic acid
- 10

group linked to the carbon in the 3-position 15 of the pyrazolone ring.

2. As new products mixed wool and silk textile goods dyed with a pyrazolone-azo dyestuff containing at least one carboxylic acid ester group in the dyestuff molecule, 20 said pyrazolone-azo dyestuff containing no free carboxylic acid group linked to the carbon in the 3-position of the pyrazolone ring.

In testimony whereof, we affix our signatures.

HERMANN WAGNER.  
HEINZ EICHWEDE.  
ERICH FISCHER.